

# UNITED STATES PATENT OFFICE.

LEIGHTON KRAMER, OF PHILADELPHIA, PENNSYLVANIA.

## PAINT AND VARNISH REMOVER AND PROCESS OF PREPARING THE SAME.

No. 882,947.

Specification of Letters Patent.

Patented March 24, 1908.

Application filed September 19, 1907. Serial No. 393,590.

*To all whom it may concern:*

Be it known that I, LEIGHTON KRAMER, a citizen of the United States, residing in Philadelphia, Pennsylvania, have invented certain Improvements in Paint and Varnish Removers and Processes of Preparing the Same, of which the following is a specification.

One object of my invention is to provide a compound which may be applied to surfaces from which it is desired to remove paint or varnish, and which will so act upon this paint or varnish as to soften or cut it to such an extent that it may be readily removed by scraping or by merely wiping off the surface.

It is further desired to provide a compound having the above noted qualities, which, in addition shall be solid or semi-solid and capable of remaining on vertical or inclined surfaces, so as to permit of their treatment for the removal of the softened paint or varnish at any desired time after the application of the compound.

Another object of the invention is to provide a paint and varnish remover, which, while capable of satisfactorily performing its functions as above indicated, shall have no objectionable qualities, that is to say, shall have no injurious effect on the hands of the person using it nor possess any objectionable odor.

A further object of my invention is to provide a process for the manufacture of my improved compound.

In carrying out my invention I mix one half pound of pulverized stearic acid and three quarters of a pint of lard oil, thereby forming a pasty or dough like mass. This I dissolve in a solution containing three pints of methyl or denatured alcohol, one pint of benzol or toluol, and one pint of acetone.

In place of the acetone, I may, if desired, use one pint of gasoline or one pint of carbon tetrachlorid. The resulting solution may be used by spreading it over surfaces from which it is desired to remove paint or varnish.

In such case, the mixture of stearic acid and

lard oil forms a protecting film which prevents the evaporation of those substances of the solution which tend to cut, remove or soften the paint or varnish, and this film causes the paint or varnish to remain in the softened condition for extended intervals of time, so that relatively large surfaces may have my solution applied to them for the purpose of removing paint or varnish thereon, after which it with the softened paint etc., may be removed by wiping or scraping when desired.

I claim:

1. A paint and varnish remover consisting of a fatty acid and a fatty oil in combination with a substance capable of softening or cutting paint and varnish.

2. A paint and varnish remover consisting of a fatty acid and an oil, dissolved in a solution containing alcohol, benzol and acetone.

3. A paint and varnish remover consisting of stearic acid and lard oil in a solution containing a substance capable of cutting paint or varnish.

4. A paint and varnish remover which consists of stearic acid, lard oil, an alcohol body, benzol and acetone.

5. A paint and varnish remover which consists in three pints of alcohol, one pint of benzol, one pint of acetone, one half pound of stearic acid and three quarters of a pint of lard oil.

6. The process of preparing a paint and varnish remover which consists in mixing a body of stearic acid with lard oil and dissolving the resulting mass in a solution containing an alcohol, benzol and acetone, in substantially the proportions specified.

In testimony whereof, I have signed my name to this specification, in the presence of two subscribing witnesses.

LEIGHTON KRAMER.

Witnesses:

WILLIAM E. BRADLEY,  
Jos. H. KLEIN.